

May 13, 1930.

J. H. UHRIG

1,758,483

METHOD FOR CASTING PIPES

Filed May 18, 1928



Inventor  
John H. Uhrig,  
By Francis J. Chenevers

Attorney.

## UNITED STATES PATENT OFFICE

JOHN H. UHRIG, OF BEVERLY, NEW JERSEY, ASSIGNOR TO UNITED STATES CAST IRON PIPE & FOUNDRY COMPANY, OF BURLINGTON, NEW JERSEY, A CORPORATION OF NEW JERSEY

## METHOD FOR CASTING PIPES

Application filed May 18, 1928. Serial No. 278,708.

My invention relates to the casting of cast iron pipes by the well known de Lavaud method and by machinery of the de Lavaud type in which relatively longitudinally movable molds and runners are employed, the metal being delivered to the mold through the end of the runner progressively as the mold is retracted from the runner so that the metal may be said to be delivered to the surface of the mold in a spiral coil. In the practice of this de Lavaud method it is found necessary that the mold and runner should be inclined to the horizontal in order to insure a sufficiently rapid flow of molten metal through the runner and under certain conditions the metal delivered to the mold has a tendency to move longitudinally in the mold before it sets, thereby bringing about an undesirable thickening and thinning of the casting and the object of my invention is to provide an improved method of casting said pipes by which this tendency to longitudinal movement of the metal in the mold is counteracted and a pipe of uniform thickness in its body portion is secured.

Generally speaking, my invention consists of reducing the angle of tilt of the mold and runner during the casting operation so as to counteract the tendency of the fluid to flow longitudinally in the mold to an undesirable extent, the lessening of the angle of tilt taking place during the pouring operation and as the mold is withdrawn from the runner and being within the control of the operator so that the tilt can be regulated in accordance with the condition of the molten iron flowing into the mold and, in practical operation, another important feature of my invention consists in pouring the metal into the runner at a point bearing a fixed relation to the mold into which the runner enters, thereby progressively shortening the distance through which the metal has to flow through the runner before reaching the mold. The diminution of frictional resistance to the flow of metal in the runner compensates to a large extent for the decreased tip of the runner during the process of casting. My invention will be best understood as described in connection with the drawings which are dia-

grammatic views partly in section of the de Lavaud pipe casting machine adapted for use in the practice of my improved method.

Figure 1 shows the machine in its initial inclined position with the end of the runner practically registering with the mold and pouring metal into the mold.

Figure 2 shows the machine with the tilt diminished with the runner nearly half withdrawn from the mold and about half of the casting completed, and

Figure 3 shows the machine tilted to horizontality and the runner almost entirely withdrawn from the mold.

A, A<sup>1</sup> and A<sup>2</sup> indicate supports for the frame B of the machine which is supported on the tracks or supports A, A<sup>1</sup>, by means of the wheels B<sup>1</sup>, all of the supporting tracks to be formed on arcs of concentric circles. C is a bracket extending out from the end of the frame B and supporting a runner indicated at C<sup>1</sup>, C<sup>2</sup> being the open end of the runner through which the metal issues into the mold. D is the ordinary water box carriage of a de Lavaud pipe casting machine, longitudinally movable on the frame B and supported thereon by wheels indicated at D<sup>1</sup>. E is the centrifugal mold rotatably supported in the water box carriage having, as shown, a bell indicated at E<sup>1</sup>. F is a ladle supporting carriage longitudinally movable on the frame B and supported thereon by wheels indicated at F<sup>1</sup>. G is a ladle supported on the carriage F and G<sup>1</sup> a runner by which the metal from the ladle is delivered to the runner C<sup>1</sup>. H indicates the casting in process of formation in the mold, H<sup>1</sup> indicating the bell end of the casting. I and I<sup>1</sup> indicate an electro-magnet and armature attached respectively to the carriage F and the mold carriage D, by means of which the carriage F is coupled to the mold carriage at such times in the operation of the machine as it is desirable that they should be coupled and moved together. J, J, indicate a horizontal level line.

It will be understood, of course, that the usual mechanism for rotating the mold and for tipping the ladle would be employed and that some convenient mechanism should be employed for shifting the carriage D on its

supporting track so as to vary its angle of inclination.

In operation the mold is first tilted to its maximum extent, as shown in Figure 1. The carriage F is coupled to the mold carriage and the ladle G gradually tilted so that metal will flow through it through the runner G into the runner F and from the end of the runner F into the bell end of the mold, as indicated in Figure 1. During the pouring the mold is moved toward the left and the operator decreases the tilt of the frame and supported parts as the pouring progresses and to such extent as, depending on the fluidity of the metal entering the mold, is necessary to prevent any objectionable longitudinal flow of the metal. As the pouring proceeds the ladle carriage F remains relatively stationary with regard to the mold so that the flow of metal through the runner E is constantly lessened, the diminution of frictional resistance to the flow of metal compensating to a great extent for the diminished angle of inclination of the runner and the spigot end of the pipe can be poured with the mold practically in horizontal position.

The mechanism diagrammatically illustrated in the figures of the drawing has been designed by me as especially well adapted for the practise of my improved method of casting pipes and its novel features form the subject matter of my co-pending application filed May 18, 1928, Serial Number 278,707. It will be understood, however, that my method is independent of any particular mechanism by means of which it is carried into effect.

Having now described my invention, what I claim as new and desire to secure by Letters Patent, is:

1. In the operation of a centrifugal pipe casting machine comprising a centrifugal mold normally inclined to a horizontal plane and a relatively longitudinally movable inclined runner through the end of which molten metal is delivered to the rotating mold as the runner is progressively withdrawn therefrom, the improved method of counter-acting the tendency to longitudinal flow of the metal in the mold which consists in decreasing the tilt of the mold and of the runner during the pouring of the metal and as the runner is withdrawn from the mold.

2. In the operation of a centrifugal pipe casting machine comprising a centrifugal mold normally inclined to a horizontal plane and a relatively longitudinally movable inclined runner through the end of which molten metal is delivered to the rotating mold as the runner is progressively withdrawn therefrom, the improved method of counter-acting the tendency to gravitational flow of the metal in the mold which consists in decreasing the tilt of the mold and of the runner during the pouring of the metal and as the run-

ner is withdrawn from the mold and by pouring the molten metal into the runner during the casting of the pipe at a point close to the end of the mold through which the runner enters the mold.

JOHN H. UHRIG.

70

75

80

85

90

95

100

105

110

115

120

125

130